

## 1

2,695,879

## ANTIFOAMANT COMPOSITION

John Adam Jehle, Jr., Media, Pa., assignor to Socony-Vacuum Oil Company, Incorporated, a corporation of New York

No Drawing. Application January 16, 1953,  
Serial No. 331,735

12 Claims. (Cl. 252—46.7)

This invention relates to the reduction of the foaming tendencies of mineral lubricating oils. It is more particularly concerned with providing extreme pressure lubricating oils having little or no tendency to form a stable foam.

As is well known to those familiar with the art, many lubricating oils have marked tendencies to foam while in use. If the foam is of a stable nature, there is a danger that it will eventually displace the lubricating oil in the lubrication system. As a consequence, circulation of sufficient lubricant will be poor, and, more seriously, there will be insufficient lubricant available to lubricate bearing surfaces, and the like. Foaming is most pronounced in lubricating oils used under extreme pressure conditions, particularly in oils for lubricating hypoid gears in motor vehicles. During operation of such vehicles, the rapid movement of the gears tends to aerate the oil. If a stable foam is formed, insufficient oil is available to lubricate the gear teeth. Most gear oils, per se, tend to foam. However, the foaming tendencies thereof are often greatly enhanced by the addition of additives for the purpose of increasing film strength, i. e., the extreme pressure additives.

It has now been found that the foaming tendencies of mineral lubricating oils can be sharply reduced, economically and simply. It has now been discovered that the foaming tendencies of mineral lubricating oils can be reduced to a minimum by adding thereto minor amounts of certain monoesters of sorbitol anhydrides, or polyoxyethylene derivatives thereof, and of the reaction product of an alkyl phenol and  $P_2O_5$ , within a critical range of ratios by weight.

Accordingly, it is a broad object of the present invention to provide non-foaming mineral lubricating oils. Another object is to provide a combination of certain monoesters of sorbitol anhydrides or polyoxyethylene derivatives thereof with the reaction product of an alkyl phenol and  $P_2O_5$ , in critical ratios, which combination eliminates foaming tendencies of mineral lubricating oils. A further object is to provide a non-foaming mineral lubricating oil containing a minor amount of this critical combination of additives. A specific object is to provide a non-foaming extreme pressure lubricant containing minor amounts of the aforementioned combination of additives. Other objects and advantages of the present invention will become apparent to those skilled in the art, from the following detailed description.

The present invention provides a mineral lubricating oil containing between about 0.1 per cent and about 1.5 per cent, by weight, of an antifoamant composition consisting of between about 2 per cent and about 30 per cent, by weight, of an ester selected from the group consisting of aliphatic monoesters of sorbitol anhydrides and aliphatic monoesters of polyoxyethylene derivatives of sorbitol anhydrides, and between about 98 per cent and about 70 per cent, by weight, of the reaction product formed by reacting about 3 moles of an alkyl phenol having a total of between about 8 carbon atoms and 12 carbon atoms in the alkyl radicals thereof, with about 1 mole of phosphorus pentoxide, at a temperature of between about 75°C. and about 125°C.

In general, any mineral lubricating oil which has foam forming tendencies is improved by the addition of the compositions of this invention. Depending upon the intended application of the lubricant, the viscosity of the oil can vary from about 1 to about 10,000 centistokes at 100°F. The extreme pressure lubricating oils are

## 2

especially preferred. These oils usually have viscosities of between about 10 and about 1500 centistokes at 100°F.

The ester additives utilizable in the antifoamant compositions of this invention are fatty acid esters of hexitans and hexides obtained by dehydrating sorbitol, and certain polyoxyethylene derivatives thereof. The compounds contemplated are known as "Spans" and "Tweens," which are manufactured by the Atlas Powder Company, Wilmington, Delaware. According to the manufacturer's literature, these esters are prepared by first dehydrating sorbitol to produce a mixture of hexitans and hexides having the following formula:



This mixture of hexitans and hexides is then esterified by reacting it with one or more moles of a fatty acid to form the "Spans." The "Tweens" are similar thereto except that the unesterified hydroxy groups in the hexitans and hexides have polyoxyethylene chains added thereto. It has been found that only the monoesters of fatty acids having between 12 and 18 carbon atoms are effective. In other words, the di- and tri-esters, and even the lower and higher monoesters, are not effective. For purposes of brevity, these esters, throughout the specification and claims, will be referred to as fatty acid monoesters of sorbitol anhydrides and polyoxyethylene derivatives thereof. Non-limited examples of the esters contemplated herein are sorbitol anhydride monolaurate, sorbitol anhydride monomyristate, sorbitol anhydride monopalmitate, sorbitol anhydride monostearate, sorbitol anhydride mono-oleate, sorbitol anhydride monolinoleate, and polyoxyethylene derivatives of the foregoing monoesters. Further data on the monoesters utilizable herein are attainable in a brochure entitled "Atlas Surface Active Agents" published in 1948 by the manufacturers, supra. Reference should be made thereto, and it is considered to be a part of this specification.

The alkylphenol- $P_2O_5$  reaction products used in the compositions of this invention are the reaction products produced by reacting an alkylphenol with phosphorus pentoxide in a molar proportion of about 3:1, respectively. The phenol reactant can be a mono- or a poly-alkyl phenol, provided that the total number of carbon atoms in the alkyl radicals is at least 8 and not more than 12. The alkyl groups can be straight chained or branched chained in structure. Furthermore, if the phenol reactant is a polyalkylated phenol, the alkyl groups can be like groups or unlike groups. Non-limiting examples of the alkylphenol reactants are dibutylphenol, di-*t*-amylphenol, di-*n*-hexylphenol, amylpropylphenol, di-secondary-amylphenol, *t*-octylphenol, trisopropylphenol, nonylphenol, decylphenol, and dodecylphenol.

The reaction between the alkylphenol reactant and  $P_2O_5$  is usually carried out at temperatures of between about 75°C. and about 125°C. The time of reaction will vary from about one hour to about 15 hours, depending upon the particular reactants used. Examples of the preparation of the reaction products contemplated herein are set forth in the co-pending application of Otto et al., Serial Number 143,156, filed February 8,

1950, now matured into U. S. Patent No. 2,638,447, issued May 12, 1953. It must be noted, however, that alkylphenol-P<sub>2</sub>O<sub>5</sub> reaction products having more than 12 carbon atoms in the alkyl groups in the alkylphenol are not utilizable herein. Thus reaction products made from tetradecylphenol and from "wax phenol" were found unsatisfactory for the purposes of the present invention.

The antifoamant compositions of this invention consist of the monoester of sorbitol anhydrides and an alkylphenol-P<sub>2</sub>O<sub>5</sub> reaction product, as defined hereinbefore. These compositions must contain between about 2 per cent and about 30 per cent, by weight, of the monoester of dehydrated sorbitol. The balance, i. e., between about 98 per cent and about 70 per cent, by weight, is the alkylphenol-P<sub>2</sub>O<sub>5</sub> reaction product. In other words, the weight ratio of the monoester to the alkylphenol-P<sub>2</sub>O<sub>5</sub> reaction product must fall within the range of between about 2:98, respectively, and about 30:70, respectively, i. e., between about 0.02 and about 0.43. Combinations having ratios outside these limits are ineffective in the present invention.

The amount of the aforescribed combinations which is added to the lubricating oil will vary between about 0.1 per cent and about 1.5 per cent, by weight. Concentrations below 0.1 per cent are effective to some extent. However, substantially complete elimination of foaming tendencies is not achieved at these concentrations.

It must be strictly understood that the non-foaming oil compositions of this invention can be produced in two ways. By one method, the dehydrated sorbitol monoester and the alkylphenol-P<sub>2</sub>O<sub>5</sub> reaction product can be blended together in the aforescribed ratios, and the resulting combination added to the mineral lubricating oil in the concentrations set forth hereinbefore. Alternatively, the monoester and the alkylphenol-P<sub>2</sub>O<sub>5</sub> reaction product can be added to the oil individually, provided, however, that they are ultimately present in the oil in the ratios set forth hereinbefore, and that the combined concentration falls within the aforescribed range. When added separately, the monoester of sorbitol anhydride is added to the oil at concentrations between about 0.002 per cent and about 0.45 per cent, by weight. Similarly, the alkylphenol-P<sub>2</sub>O<sub>5</sub> reaction product is added to the oil at concentrations of between about 0.07 per cent and about 1.47 per cent, by weight. It is very important, however, when working within these ranges, (1) that the ratio of ester to reaction product be maintained, and (2) that the combined concentrations fall within the range set forth hereinbefore. Thus, for example, 0.002 weight per cent of sorbitol anhydride mono-oleate added to an oil containing 0.5 weight per cent of the di-*t*-amylphenol-P<sub>2</sub>O<sub>5</sub> reaction product is ineffective. Although the concentrations of the additives in this blend fall within the ranges specified, it will be noted that the ratio of the mono-oleate to the reaction product was only about 0.4:99.6, i. e., about 0.004. Since the ratio must fall within the range of between about 2:98 and about 30:70, i. e., between about 0.02 and about 0.43, it will be appreciated that the ratio in this case, is outside the effective range.

A preferred embodiment of the present invention is a non-foaming extreme pressure lubricating oil. Since the alkylphenol-P<sub>2</sub>O<sub>5</sub> reaction products impart extreme pressure characteristics to lubricating oils, they are frequently used as at least one component thereof. However, in order to achieve good extreme pressure properties in an oil, the alkylphenol-P<sub>2</sub>O<sub>5</sub> reaction product should be present in somewhat larger amounts than set forth hereinbefore, namely, at concentrations of about 0.1 per cent and 1.5 per cent, by weight. A preferred concentration is about 0.5 per cent. Accordingly, in order to render these extreme pressure oils non-foaming, the sorbitol anhydride monoester will be added at concentrations of between about 0.002 per cent and about 0.45 per cent, by weight. When operating within these ranges, the ratios defined hereinbefore must be maintained. The concentration of the anti-foamant combination present in these oil compositions will be between about 0.1 per cent and about 2.5 per cent, by weight. An improved extreme pressure lubricating oil of the type contemplated within the preferred embodiment of this invention is disclosed in the Otto et al. co-pending application, Serial Number 143,156, filed February 8, 1950, now matured into U. S. Patent No. 2,638,447, issued May 12, 1953. Briefly described, these mineral lubricating oils contain (1) be-

tween about one per cent and about 10 per cent, by weight, of a product obtained by chemically substituting a part only of the chlorine in a chlorinated aliphatic material with a thiocarbonate group, (2) between about 0.1 per cent and about 3 per cent, by weight, of dihydroabietyl malate, and (3) between about 0.1 per cent and about 1.5 per cent by weight of an alkylphenol-P<sub>2</sub>O<sub>5</sub> reaction product. Reference should be made to this application for details of the compositions contemplated. These compositions have excellent extreme pressure properties. They do, however, exhibit a tendency to foam. Such compositions are rendered non-foaming by the present invention. As disclosed in the Otto et al. application, the alkylphenol can have a total of less than eight and more than twelve carbon atoms in the alkyl groups for extreme pressure purposes. Thus, for example, a wax-alkylated phenol-P<sub>2</sub>O<sub>5</sub> reaction product is operable as an extreme pressure agent. In such a case, another alkylphenol-P<sub>2</sub>O<sub>5</sub> reaction product within the ranges contemplated herein must be added with the sorbitol anhydride monoester to achieve non-foaming characteristics.

The effectiveness of the antifoamant compositions of this invention is not impaired by the presence of other additives in the lubricating oil blend. The non-foaming oil compositions of this invention can contain a wide variety of other oil addition agents for the purpose of improving other characteristics of the oil. Accordingly, extreme pressure addition agents, antirust agents, oiliness agents, pour point depressants, detergents, and the like, well known to those skilled in the art, can be added to a lubricating oil along with the antifoamant compositions of this invention.

Oil concentrates are also contemplated herein. Thus, blends containing upwards of 1.5 per cent, as much as about 49 per cent, by weight, of the antifoamant compositions of this invention in a suitable lubricating oil can be used. These concentrates can subsequently be diluted with a base oil, in order to achieve an ultimate blend containing the desired concentration of the antifoamant composition.

The following specific examples are for the purpose of illustrating the antifoamant compositions of this invention. It must be strictly understood that this invention is not to be limited to the specific fatty acid monoesters of sorbitol anhydrides and polyoxyethylene derivatives thereof, and to the alkylphenol-P<sub>2</sub>O<sub>5</sub> reaction products disclosed therein, or to the concentrations used. As will be apparent to those skilled in the art, other monoesters of sorbitol anhydride and alkylphenol-P<sub>2</sub>O<sub>5</sub> reaction products, and other concentrations thereof can be used, as has been fully disclosed hereinbefore.

The test procedure used to determine the foaming characteristics of the lubricating oil is the CRC foam test, designation L-14, which is described in the CRC handbook. In brief, this test involves blowing air through a sample of the oil under test at 75° F. for 5 minutes. The sample is contained in a graduated cylinder. At the end of the blowing period, the volume of foam is noted. The volume of foam at the end of a 10-minute collapse period, as was called for in the test, is not reported herein. The non-foaming oils of this invention show virtually no foam at the end of the blowing period, thus no collapse period is required.

The base oil used to illustrate the compositions of this invention is a solvent-refined residual oil. This oil has an A. P. I. gravity of about 27.5, a Saybolt universal viscosity of 1075 at 100° F. and 90-95 at 212° F., a pour point of +25° F., and a fraction point of 460° F.

In the following examples commercially available, Spans and Tweens were used. Of the materials tested, "Span 80" is defined as sorbitol anhydride mono-oleate, "Span 85" is sorbitol anhydride trioleate, "Tween 21" is polyoxyethylene sorbitol anhydride mono-laurate, "Tween 61" is polyoxyethylene sorbitol anhydride mono-stearate, "Tween 81" is polyoxyethylene sorbitol anhydride mono-oleate. Other identifying characteristics of these materials can be obtained from the manufacturer's brochure identified hereinbefore.

#### Examples 1. through 3

Three lubricating oil blends were subjected to the foaming test. The first blend comprised about 0.2 per cent Tween 81 in the test oil. The second blend comprised the test oil containing about 0.1 per cent Tween 81 and about 0.5 per cent of the reaction product of 3 moles of di-*t*-amylphenol with 1 mole of phosphorus pentoxide. The

third blend comprised the base oil containing about 0.01 per cent Tween 81 and about 0.5 per cent of the amylphenol-P<sub>2</sub>O<sub>5</sub> reaction product. Pertinent data and test results therefor are set forth in the table.

*Examples 5 through 8*

Two portions of the base oil containing 0.5 per cent by weight of the reaction products of 3 moles of di-t-amylphenol with 1 mole of phosphorus pentoxide were blended with varying amounts of Tween 61 and Tween 21. Pertinent data on these blends and foam test results therefor are set forth in the table.

*Example 4*

An extreme pressure lubricating oil composition was prepared by blending in the base oil 5 per cent by weight of a chlorinated xanthate produced by reacting chlorinated kerosene with sodium ethyl xanthate, 1 per cent by weight of di-hydroabietyl malate, 0.5 per cent by weight of the alkylphenol-P<sub>2</sub>O<sub>5</sub> reaction product of Examples 1 through 3, and 0.2 per cent by weight of Tween 81. This composition, when subjected to the foaming test, gave the results as set forth in the table.

*Example 9*

In the base oil were blended 0.2 per cent by weight of Span 80 and 0.5 per cent by weight of the alkylphenol-P<sub>2</sub>O<sub>5</sub> reaction product of the preceding example. This blend, when subjected to the foam test, gave the results set forth in the table.

*Example 10*

An extreme pressure lubricating oil composition was prepared by blending in the base oil 5 per cent by weight of a chlorinated xanthate produced by reacting chlorinated kerosene with sodium ethyl xanthate, 1 per cent by weight of di-hydroabietyl malate, 0.5 per cent by weight of the alkylphenol-P<sub>2</sub>O<sub>5</sub> reaction product of Examples 1 through 3, and 0.2 per cent by weight of Span 80. This composition, when subjected to the foaming test, gave the results as set forth in the table.

*Example 11*

For purposes of comparison, a blend was prepared comprising 0.2 per cent by weight of Span 85 and 0.5 per cent by weight of the reaction product of 3 moles of octylphenol (mixed isomers) with 1 mole of phosphorus pentoxide in the base oil, as will be apparent from the data set forth in the table. This blend foamed appreciably in the foaming test.

It will be appreciated, from the foregoing examples, that combinations of sorbitol anhydride monoesters with certain alkylphenol-P<sub>2</sub>O<sub>5</sub> reaction products eliminate the foaming tendencies of mineral oils, when added thereto in definite amounts and in definite proportions. Likewise, standard gear oil formulations containing other E. P. additives are beneficiated in that respect. It is to be noted that the ester of the sorbitol anhydride must be a monoester and must contain between 12 and 18 carbon atoms in the acid radical.

Although the present invention has been described with preferred embodiments, it is to be understood that modifications and variations may be resorted to without departing from the spirit and scope thereof, as those skilled in the art will readily understand. Such variations and modifications are considered to be within the purview and scope of the appended claims.

TABLE

| Exam-<br>ple | Conc. of<br>Comp., Wt.<br>Percent | A <sup>1</sup>  | B <sup>2</sup> | Wt.<br>Ratio,<br>A/B <sup>3</sup> | Foam,<br>ml. |
|--------------|-----------------------------------|-----------------|----------------|-----------------------------------|--------------|
|              | Blank oil.                        |                 |                |                                   | 400-600      |
| 1            | 0.2                               | Tween 81        | None           |                                   | 470          |
| 2            | 0.6                               | do              | diamylphenol   | 16.7:83.3                         | nil          |
| 3            | 0.51                              | do              | do             | 2.98                              | 10           |
| 4            | 0.7                               | do              | do             | 28.6:71.4                         | nil          |
| 5            | 0.6                               | Tween 61        | do             | 16.7:83.3                         | nil          |
| 6            | 0.51                              | do              | do             | 2.98                              | nil          |
| 7            | 0.6                               | Tween 21        | do             | 16.7:83.3                         | nil          |
| 8            | 0.51                              | do              | do             | 2.98                              | nil          |
| 9            | 0.7                               | Span 80         | do             | 28.6:71.4                         | nil          |
| 10           | 0.7                               | do <sup>4</sup> | do             | 28.6:71.4                         | nil          |
| 11           | 0.7                               | Span 85         | octylphenol    | 28.6:71.4                         | 170          |

<sup>1</sup> A = Sorbitol anhydride monoester or polyoxyethylene derivative.

<sup>2</sup> B = Alkylphenol reacted with P<sub>2</sub>O<sub>5</sub> in a 3:1 molar proportion.

<sup>3</sup> B' = Alkylphenol-P<sub>2</sub>O<sub>5</sub> reaction product.

<sup>4</sup> Plus 5% chlorinated xanthate and 1% dihydroabietyl malate.

What is claimed is:

1. A mineral lubricating oil containing between about 0.1 per cent and about 1.5 per cent, by weight, of an antifoam composition consisting of between about 2 per cent and about 30 per cent, by weight, of an ester selected from the group consisting of aliphatic monoesters of sorbitol anhydrides and aliphatic monoesters of polyoxyethylene derivatives of sorbitol anhydrides, and between about 98 per cent and about 70 per cent, by weight, of the reaction product formed by reacting about 3 moles of an alkyl phenol having a total of between about 8 carbon atoms and about 12 carbon atoms in the alkyl radicals thereof, with about 1 mole of phosphorus pentoxide, at a temperature of between about 75° C. and about 125° C.
2. A mineral lubricating oil containing between about 0.1 per cent and about 1.5 per cent, by weight, of an antifoam composition consisting of between about 2 per cent and about 30 per cent, by weight, of sorbitol anhydride mono-oleate and between about 98 per cent and about 70 per cent, by weight, of the reaction product formed by reacting about 3 moles of diamylphenol with about 1 mole of phosphorus pentoxide, at a temperature of between about 75° C. and about 125° C.
3. A mineral lubricating oil containing between about 0.1 per cent and about 1.5 per cent, by weight, of an antifoam composition consisting of about 17 per cent, by weight, of sorbitol anhydride mono-oleate and about 83 per cent, by weight, of the reaction product formed by reacting about 3 moles of diamylphenol with about 1 mole of phosphorus pentoxide, at a temperature of between about 75° C. and about 125° C.
4. A mineral lubricating oil containing between about 0.1 per cent and about 1.5 per cent, by weight, of an antifoam composition consisting of between about 2 per cent and about 30 per cent, by weight, of sorbitol anhydride mono-oleate and between about 98 per cent and about 70 per cent, by weight, of the reaction product formed by reacting about 3 moles of diamylphenol with about 1 mole of phosphorus pentoxide, at a temperature of between about 75° C. and about 125° C.
5. A mineral lubricating oil containing between about 0.1 per cent and about 1.5 per cent, by weight, of an antifoam composition consisting of about 2 per cent, by weight, of sorbitol anhydride mono-oleate and about 98 per cent, by weight, of the reaction product formed by reacting about 3 moles of di-amylphenol with about 1 mole of phosphorus pentoxide, at a temperature of between about 75° C. and about 125° C.
6. A mineral lubricating oil containing between about 0.1 per cent and about 1.5 per cent, by weight, of an antifoam composition consisting of between about 2 per cent and about 30 per cent, by weight, of sorbitol anhydride monolaurate and between about 98 per cent and about 70 per cent, by weight, of the reaction product formed by reacting about 3 moles of di-amylphenol with about 1 mole of phosphorus pentoxide, at a temperature of between about 75° C. and about 125° C.
7. A mineral lubricating oil containing between about 0.1 per cent and about 1.5 per cent, by weight, of an antifoam composition consisting of about 2 per cent, by weight, of sorbitol anhydride monolaurate and about 98 per cent, by weight, of the reaction product formed by reacting about 3 moles of di-amylphenol with about 1 mole of phosphorus pentoxide, at a temperature of between about 75° C. and about 125° C.
8. A mineral lubricating oil containing between about 0.1 per cent and about 1.5 per cent, by weight, of an antifoam composition consisting of between about 2 per cent and about 30 per cent, by weight, of polyoxyethylene sorbitol anhydride mono-oleate and between about 98 per cent and about 70 per cent, by weight, of the reaction products formed by reacting about 3 moles of di-amylphenol with about 1 mole of phosphorus pentoxide, at a temperature of between about 75° C. and about 125° C.
9. A mineral lubricating oil containing between about 0.1 per cent and about 1.5 per cent, by weight, of an antifoam composition consisting of about 29 per cent, by weight, of polyoxyethylene sorbitol anhydride mono-oleate and about 71 per cent, by weight, of the reaction product formed by reacting about 3 moles of di-amylphenol with about 1 mole of phosphorus pentoxide, at a temperature of between about 75° C. and about 125° C.

10. A mineral lubricating oil containing (1) between about 0.1 per cent and about 1.5 per cent, by weight, of an antifoamant composition consisting of between about 0.1 per cent and about 30 per cent, by weight, of an aliphatic monoester of polyoxyethylene sorbitol anhydride, and between about 98 per cent and about 70 per cent, by weight, of the reaction product formed by reacting about 3 moles of an alkyl phenol having a total of between about 8 carbon atoms and about 12 carbon atoms in the alkyl radicals thereof, with about 1 mole of phosphorus pentoxide, at a temperature of between about 115° C. and about 125° C.; (2) between about 1 per cent and about 10 per cent, by weight, of a product obtained by chemically substituting a part only of the chlorine of a chlorinated aliphatic hydrocarbon material having from 2 to about 24 carbon atoms with a diocarbonate group; and (3) between about 0.1 per cent and about 3 per cent, by weight, of dihydroabietyl malate.

11. The composition defined in claim 10 wherein the aliphatic monoester of polyoxyethylene sorbitol anhydride is polyoxyethylene sorbitol anhydride mono-oleate and the alkyl phenol is di-*amylphenol*.

12. A mineral lubricating oil containing (1) between about 0.1 per cent and about 1.5 per cent, by weight, of an antifoamant composition consisting of about 29 per cent, by weight, of polyoxyethylene sorbitol anhy-

dride mono-oleate and about 71 per cent, by weight, of the reaction product formed by reacting about 3 moles of di-*amylphenol* with about 1 mole of phosphorus pentoxide, at a temperature of between about 75° C. to about 125° C.; (2) about 5 per cent, by weight, of a product obtained by chemically substituting a part only of the chlorine in a chlorinated petroleum naphtha with an alkyldi-*xanthate* group; said product having a chlorine content of from about 25 per cent to about 40 per cent and a *xanthate* group content of about 10 per cent to about 22 per cent; and (3) about 1 per cent, by weight, of dihydroabietyl malate.

#### References Cited in the file of this patent

#### UNITED STATES PATENTS

| Number    | Name        | Date          |
|-----------|-------------|---------------|
| 2,418,422 | Palmer      | Apr. 1, 1947  |
| 2,603,599 | Trautman    | July 15, 1952 |
| 2,622,066 | Jehle       | Dec. 16, 1952 |
| 2,638,447 | Otto et al. | May 12, 1953  |

#### OTHER REFERENCES

Foaming of Aircraft Engine Oils as a Problem in Colloid Chemistry—I. NACA report, ARR. No. 4105, originally issued September 1944, declassified April 26, 1946, pg. 73 pertinent.